

## UNITED STATES PATENT OFFICE

2,056,591

ARTICLES WITH REDUCED TENDENCY  
TO CORRODE

Hermann Schulz and Carl Carius, Dortmund,  
Germany, assignors to the firm Vereinigte  
Stahlwerke Aktiengesellschaft, Dusseldorf,  
Germany

No Drawing. Original application May 31, 1933,  
Serial No. 673,792. Divided and this applica-  
tion June 30, 1936, Serial No. 88,267. In Ger-  
many May 20, 1932

## 1 Claim. (Cl. 75—124)

The invention relates to articles made from steel and cast iron with reduced tendency to corrode, especially when subjected to the action of water, especially sea water and moist soil, and 5 forms a division from my co-pending application Serial No. 673,792, filed May 31, 1933.

The present invention is an improvement of the steel and cast iron described and claimed by the applicant in his prior application Serial Number 450,878, which matured into Patent No. 2,013,-  
10 600 on Sept. 3, 1935, which is also resistant against sea water and moist soil. The prior process is based upon special electrolytic actions which are thereby caused, that the steel or cast iron is al-  
15 loyed with copper, antimony, arsenic, or tin and in combination with one or several of these ad-  
ditions with magnesium, nickel or aluminium. Said elements are used in the prior process in the following amounts: antimony, arsenic, tin in  
20 amounts between 0.05 and 5%, singly or together, copper in amounts up to 1%, magnesium be-  
tween 0.1 and 5%, aluminum between 0.05 and 5%.

Further researches have shown that the titani-  
25 um and vanadium elements act in a similar way as the magnesium and aluminum elements used secondly according to the main patent, and they are not only equivalent to these elements, especially aluminium, but even superior thereto.  
30 Since this has been found out, it is possible to replace the aluminum as well as magnesium partly by titanium or vanadium. The favourable in-  
fluence of these two elements could not be fore-  
seen either on account of their electrochemical  
35 or chemical behaviour.

A further economically advantageously acting influence of titanium and vanadium, owing to which steels alloyed with these elements will excel compared with aluminum containing steels, is  
40 that the capacity of steels alloyed with titanium and vanadium of offering increased resistance to the attacks of water will find expression already a short time after the beginning of corrosion in a considerable reduction of corroding speed. For  
45 example the corroding speed in sea water will be reduced already after 14 days approximately 20% and in river water about 40% compared with that of copper-nickel steels alloyed with aluminum. Steels according to the invention are further dis-  
50 tinguished by a perfectly uniform rusting of their surface exposed to the corroding agent. Local corrosion attacks in the form of dents or holes or notch-like depressions, which cause a reduc-  
55 tion of the mechanical qualities of a steel, do not happen. From the point of view of foundry

technics and metallurgy too, the possibility of partly substituting titanium or vanadium for aluminum affords an advantage in so far as steels mixed with titanium and vanadium can be worked better than those having a high addition of 5 aluminum.

The two elements will have the effect described already at very slight amounts thereof, namely, of both metals together are present in a quantity of 10 0.1%. Upwardly, the amount of metals with re-  
spect to their corrosion-stopping influence is un-  
limited. However, it is advisable when adding  
15 titanium not to exceed 1% and in case of vanadi-  
um 0.5%, as a greater addition would not afford any extra advantages.

Thus the invention comprises articles with a reduced tendency to corrode under the action of a corroding agent, more particularly the moisture contained in water, seawater and moist soil; said articles being made from a ferrometal alloy con-  
20 taining 0.2-1% copper, titanium between about 0.1 and 1%, vanadium between about 0.1 and 0.5% and in addition aluminum in amounts be-  
25 tween about 0.05 and 3% and the balance sub-  
stantially all iron, the alloying elements copper and aluminum forming together with titanium and vanadium a firmly adhering skin on the ar-  
30 ticles, due to the corroding attack by said cor-  
roding agent.

It may be mentioned that the further composi-  
35 tion of the alloys besides the elements above speci-  
fied is the usual one. Thus the alloy may be al-  
loyed for some other reasons with the usual  
amounts of elements such as for example manga-  
35 nese, silicon, phosphorus, chromium, tungsten,  
molybdenum, cobalt, boron, zirconium, beryllium,  
as has been stated in my prior patent and in the  
case of steels the accompanying elements may be  
40 present in approximately the following amounts:

|                 | Per cent          |
|-----------------|-------------------|
| Carbon-----     | Traces up to 1    |
| Silicon-----    | Traces up to 0.5  |
| Manganese-----  | 0.1 to 1          |
| Sulphur-----    | Traces up to 0.12 |
| Phosphorus----- | Traces up to 0.2  |

45 and in the case of iron in approximately the fol-  
lowing amounts:

|                 | Per cent          |
|-----------------|-------------------|
| Carbon-----     | 2 to 3.6          |
| Silicon-----    | 0.3 to 3          |
| Manganese-----  | 0.3 to 1.2        |
| Sulphur-----    | Traces up to 0.12 |
| Phosphorus----- | Traces up to 1.0  |

50 55

We claim:

Articles with a reduced tendency to corrode under the action of a corroding agent, more particularly the moisture contained in water, sea-water and moist soil; said articles being made from a ferrometal alloy containing 0.2-1% copper, vanadium in amounts between about 0.1 and 0.5%, titanium between about 0.1 and 0.5% and in addi-

tion aluminum in amounts between about 0.05 and 3% the balance substantially all iron, the alloying elements copper and aluminum forming together with titanium and vanadium a firmly adhering skin on the articles, due to the corroding attack 5 by said corroding agent.

HERMANN SCHULZ.  
CARL CARIUS.